

# UNITED STATES PATENT OFFICE.

RHETHERFORD B. MARTIN, OF NEW YORK, N. Y., ASSIGNOR TO MINERALS SEPARATION  
NORTH AMERICAN CORPORATION, OF NEW YORK, N. Y., A CORPORATION OF MARY-  
LAND.

## ORE CONCENTRATION.

1,236,856.

Specification of Letters Patent. Patented Aug. 14, 1917.

No Drawing.

Application filed January 28, 1916. Serial No. 74,921.

To all whom it may concern:

Be it known that I, RHETHERFORD B. MARTIN, a citizen of the United States, residing at the borough of Manhattan, in the county 5 of New York and State of New York, have invented certain new and useful Improvements in Ore Concentration, of which the following is a specification.

This invention consists in improvements 10 in processes of ore concentration, and has particular reference to the concentration of ores by flotation. In these processes the powdered ore is usually mixed with water, such mixture being termed the pulp, and to 15 this pulp is added the frothing agent, consisting of an oil or oils or a soluble frothing agent or agents, or both, and the pulp is then subjected to agitation and aeration, for example, supra-aeration by air introduced 20 from above by beating it into the pulp, or subaeration by air introduced from below through a porous medium or otherwise, as well known in the art, the result of this aeration and agitation being that the air 25 bubbles coursing through the pulp gather up the metalliferous particles and carry them to the surface where they form a froth. This froth may be readily floated over a lip or dam, and will thus carry the 30 metalliferous particles away from the body of the liquid. In these processes a mineral acid, such as sulfuric acid, is in some instances used in addition to the frothing agent, and in other instances an alkali is 35 used in addition to the frothing agent, and these additional substances, acid or alkaline, act in some manner not clearly understood to modify the properties of the liquid and to assist the flotation of the metalliferous 40 mineral and to retard or prevent the flotation of the gangue.

I have found that soluble sulfids, such as mono-sulfids, polysulfids or hydrosulfids of sodium, potassium and calcium, are 45 capable of use for this purpose, that is to say, to modify the properties of the liquid forming the pulp so that the selective action of the frothing agent and air bubbles is enhanced or usefully influenced, and that by 50 their use in the proportions and under the conditions hereinafter stated, not only may improved concentration be effected of the metalliferous sulfid particles, such as have hitherto been concentrated in flotation proc-

esses, but also concentration may be effected 55 of oxidized metalliferous particles, such as oxids and carbonates of copper.

It has hitherto been proposed to treat oxidized metalliferous particles with soluble sulfids under such conditions that the oxidized metalliferous particles are converted into or become superficially coated with metallic sulfids and are thereby rendered suitable for concentration by flotation, as in British Patent No. 26,019 of 1909, to 60 Sulman and Picard. The procedure according to my invention is wholly different from that heretofore proposed, in that the oxidized metallic particles are not converted into or coated with sulfid particles, but are 65 selected and concentrated as oxidized particles. For example, if the ore contains particles of carbonates of copper, of the malachite variety, green in color, these copper carbonate particles remain particles of copper carbonates throughout the process and are clearly recognizable as particles of green copper carbonates in the concentrates. I have further found that if the amount of 70 soluble sulfid is increased above the minute 75 quantities which I have successfully used, or if the duration of its contact with the copper carbonates is extended, or if heat is used, so as in any one or all of these instances to coat the green copper carbonate 80 particles with the sulfid of copper produced by such conversion, which is black, that the 85 process is seriously impaired and that as the condition of conversion into copper sulfid is approached the impairment of the 90 process increases and in some instances useful froth formation is prevented.

The sulfid solution may be prepared by dissolving one or more of the commercial sulfids in water in suitable quantities, or it 95 may be prepared, for example, by boiling in water a mixture of sulfur and one or more alkali hydrates or alkaline earth hydrates. The following are examples of the methods last referred to of preparing sulfid solutions for use in this process.

Example 1: Boil together for a period of about ten minutes the following substances:

52 parts of caustic soda

48 parts of flowers of sulfur

6000 parts of water.

Example 2: Boil together for a period of about ten minutes—

47 parts of lime  
53 parts of flowers of sulfur  
6000 parts of water.

Example 3: Boil together for a period of 5 about fifteen minutes—

44.6 parts of lime  
50.4 parts of flowers of sulfur  
1 part of caustic soda  
6000 parts of water.

10 The resulting liquid is usually of a dark golden color when hot, and a golden yellow when cold. Some residue may be left, especially when the materials used are impure, which should be allowed to settle and the 15 clear liquid decanted; or the solution may be cleared by filtration.

In the use of this invention a small quantity of the solution, depending on the strength of the solution and on the nature of 20 the ore, is added to the pulp either before or with or after the addition of the frothing agent, and before or at the beginning of the agitation and aeration. The best results have been generally obtained by the 25 addition of the solution before the frothing agent. Further, an excess of the sulfid solution may cause coagulation of the ore slimes and may prevent the formation of a froth and is to be avoided.

30 I have found that for the treatment of 500 grams of finely powdered porphyry copper ore, containing about 2% of copper as sulfids, 10 cubic centimeters of the solution made according to Example 1 (sodium polysulfid 0.034% of the ore) in 1500 grams of water at normal temperature, may be used with a frothing agent in the proportion of one pound to the ton of ore, such frothing agent consisting of 90% gas tar creosote and 40 10% yellow pine oil. Agitation and aeration produce a mineral froth containing the copper sulfids of the ore, and the froth is floated off or separated in any suitable manner. With such treatment any copper car-

45 bonates present in the ore are concentrated with the copper sulfid and appear in the concentrates as copper carbonates; and an ore or tailings containing the copper in the form of carbonates without any copper sulfids may 50 be efficiently concentrated and the carbonates of copper will appear in the froth and will be separated as concentrates in the form of copper carbonates.

In place of the solution made according to 55 Example 1, a sulfid solution may be prepared by dissolving sodium polysulfid, commercially known as fused sodium sulfid, in the proportion of 40 grams per liter of water; and 10 cubic centimeters of this solution may be used with 1500 grams of water at normal temperature for the treatment of 60 500 grams of the ore above referred to with the frothing agent above referred to. The proportion of the polysulfid in the ore pulp

will be 0.027% of the water of the ore pulp 65 and 0.08% of the ore.

The following is an example of carrying out my process on a large scale, the material treated being mill slimes of a porphyry copper ore in a pulp containing four parts of 70 water to one of the slimes. The average assay value of the slimes was about 0.9% copper, of which 0.3% was oxidized. A solution made according to Example 3 was 75 added to the pulp in the proportion of six gallons of the solution per ton of slimes treated, and thereafter the frothing agent was added to the solution. This frothing agent contained oils modified in accordance with the process described and claimed in 80 my application for Letters Patent filed simultaneously herewith, Serial No. 74,932, and not claimed herein, that is to say, these oils had been mixed with sulfur and subjected to high temperatures, in the neighborhood of 200° to 350° centigrade, in an ordinary still, and the distillates collected for use. Prior to the distillation treatment, the pine oil had been mixed in the proportion of 100 cc. of the oil and 5 grams of 90 sulfur, and the petroleum distillate and sulfur had been mixed in like proportions. This frothing agent contained 10% of light coal tar oil, 10% of pine oil modified as above described, and 80% of a petroleum 95 distillate of 30° Baumé modified as above described, and was used in the proportion of 1.7 to 2 pounds per ton of slimes treated. Agitation and aeration produced a froth of 100 concentrates which assayed about 10% copper and tailings which assayed about 0.1% copper.

In the application of this invention to various ores and under various conditions, the examples of the process above described 105 may be modified without departing from this invention.

I claim:

1. A process of concentrating ores which consists in submitting an ore pulp to flotation separation with agitation and aeration in the presence of a soluble sulfid dissolved in the pulp in an amount and under conditions of treatment so regulated as not to coat oxidized particles with a visible layer 110 of sulfid during such treatment, and by such treatment to obtain a froth of concentrates.

2. A process of concentrating ores containing oxidized metalliferous particles which consists in submitting an ore pulp of 115 such an ore to flotation separation with agitation and aeration in the presence of a soluble sulfid dissolved in the pulp in an amount and under conditions of treatment so regulated as not to coat oxidized particles with a visible layer of sulfid during such treatment, and by such treatment to obtain 120 a froth of concentrates.

3. A process of concentrating ores containing copper which consists in submitting an ore pulp of such an ore to flotation separation with agitation and aeration in the presence of a soluble sulfid dissolved in the pulp in an amount and under conditions of treatment so regulated as not to coat oxidized particles with a visible layer of sulfid during such treatment, and by such treatment to obtain a froth of concentrates.

4. A process of concentrating ores containing oxidized copper which consists in submitting an ore pulp of such an ore to

flotation separation with agitation and aeration in the presence of a soluble sulfid dissolved in the pulp in an amount and under conditions of treatment so regulated as not to coat oxidized particles with a visible layer of sulfid during such treatment, and by such treatment to obtain a froth of concentrates.

15

In testimony whereof I have affixed my signature.

RHETHERFORD B. MARTIN.

Witnesses:

HENRY D. WILLIAMS,  
HARRY C. LEWIS.